

Jan. 17, 1939.

H. KARL

2,143,948

FUSED COATING OF SOLID METAL FOR WRAPPINGS AND OTHER  
PURPOSES, INCLUDING DECORATION, ETC

Filed Dec. 14, 1933

2 Sheets-Sheet 1



Inventor  
Heinrich Karl

Jan. 17, 1939.

H. KARL

2,143,948

FUSED COATING OF SOLID METAL FOR WRAPPINGS AND OTHER

PURPOSES, INCLUDING DECORATION, ETC

Filed Dec. 14, 1933

2 Sheets-Sheet 2



## UNITED STATES PATENT OFFICE

2,143,948

FUSED COATING OF SOLID METAL FOR  
WRAPPINGS AND OTHER PURPOSES,  
INCLUDING DECORATION, ETC.

Heinrich Karl, Jersey City, N. J.

Application December 14, 1933, Serial No. 702,344

18 Claims. (Cl. 41—18)

This invention relates to improvements in solid and sticking metal coatings for wrappers or boxes of all sorts of containers that serve for holding and preserving all kinds of goods that must be 5 protected from the influence of air, moisture, etc. I have invented also such solid metal coatings that stick to metal or non-metallic materials, such as paper, cardboard, Cellophane, wood, linoleum, glass, stone, cloth, enamel, china, 10 leather, dry paint, plaster and to all other dry matter or fabrics or materials and it may serve for a decorative purpose, as, for instance, the beautifying of the walls and ceilings of rooms or of houses or for the ornamentation of all kinds 15 of objects, such as, for instance, covers of books, doors, windows, stairs, mugs, vases, bottles and glasses, shields and signs, furniture, mirrors, caskets, etc. and it may serve also for the substantial strengthening of the coating of letters 20 and ornaments painted on glass or enamel, etc. These ornaments or decorative parts which are then covered with said aforesaid solid metal coating may be embossed before or afterward, provided the material upon which the ornaments 25 are made permit the embossing afterward. There may be also shingles, slates or other roofing and wall covering materials covered with a coating of metal for obtaining decorative effects and for making them waterproof.

30 In another application for patent having the title "Sanitary cans and the coating of them with metal" with the Serial No. 702,345 that I made jointly with the present one and filed also on December 14, 1933, the method of forming a solid 35 metal coating in sanitary preserving cans is described and claimed also and there is substantially the same process described as in the present invention that will be described now in detail and claimed subsequently.

40 In the accompanying drawings,

Figure 1 represents a partly rolled up wrapping paper to which the solid coating of metal (by preference tin) is applied thereto and which sticks to it and whereby the other side of said 45 wrapping paper is printed on;

Figure 2 shows an enlarged section through the wrapping paper of Figure 1;

Figure 3 shows in perspective view some eatable wrapped in the coated paper that has a 50 label printed on;

Figure 4 shows a few examples of the innumerable motives of ornamental and figural decorative suggestions that might serve for a room or that might ornate a door, etc., and which can be 55 made in metal in the method described herein-

after and which might also be embossed and cut out so as to give chance for colorful or contrasting backgrounds, etc.;

Figure 5 shows a diagrammatic representation of a machine in which the successive functions 5 are illustrated to which the paper, etc. must undergo until the finished product is obtained; and

Figure 6 shows the most effective method of spraying on the molten metal by means of a 10 specially constructed hot gas-spraying device.

It is customary to wrap candy, tobacco, tea and other goods in tin foil and to wrap again a paper that is printed on or that is not printed on around the tin foil or to paste a label on it. The 15 tin foil is to prevent the deterioration of the wrapped goods while the paper is mostly used for labeling the goods. In the present invention both the paper and the tin are united and through it they strengthen each other sufficiently for permitting the tin layer to be comparatively thin, which refers also to any other suitable metal. Instead of the paper there may be other materials employed, such as Cellophane and even 20 cloth that might be coated with a suitable other 25 material such as paper pulp, etc., or there may be sheets of metal or of wood employed.

The coating with metal (chiefly with tin) of these materials is made in the following described manner whereby for simplification in the description only "paper" is mentioned as the means 30 for wrapping the goods.

Referring to Figures 1, 2 and 3, the wrapping paper is indicated by 10 and the tin that sticks to it by 11. The simplest way of making that 35 kind of tinned paper is by coating the one side of a large sheet or of the whole roll 12 as it comes in its largest full size from the mill with a varnish or lacquer 13 which is best applied by a machine with special cylinder (see Figure 5) 40 whereupon the still wet coating must be bronzed similarly as is done in the printing trade. There may be taken any of the usual bronzes, but for the reduction of the cost it is advisable to use the more economical iron bronze, which is powdered 45 iron. The powdered metal sticks to the wet lacquer, etc. and forms a metallic coating which, however, is not of the desired thickness nor of such density that is necessary for rendering the wrapping or package air and watertight. It is 50 therefore necessary to add a solid metal coating by fusing it with the bronze on the side of the wrapping paper. The bronzed side of the whole sheet must then be fluxed slightly which is best and simplest made by a revolving cylinder that 55

is partly immersed in the flux and to which the bronzed side of the large sheet is pressed on whereupon other rollers or cylinders even out the flux on the bronzed surface of the sheet. Another cylinder which is partly immersed in the molten metal, preferably tin, applies the molten metal to the bronzed and then fluxed side of the paper while it revolves and while the paper travels along whereby the molten metal becomes fused with the bronze on the paper.

The paper may then be rolled up or it may be cut into large sheets or it may be cut right to the size of the single wrapping paper.

The printing of the label or of any descriptive or decorative matter on the other side of the sheet can be made before the coating is applied or it may be done afterward. If the metal coating is to be applied for decorative purposes there are several ways for making the coating.

One of the most practical methods is that to print the design on paper in the lithographic or other process and to bronze that paper whereby only the varnish or lacquer of the design will take the powdered metal. Since the bronze alone will not suffice to give the consistency that is necessary and the impression of a solid sheet or layer of metal, it is necessary to flux the sheets and to apply the molten metal thereto whereby it will stick only to the bronzed parts. The molten metal may be blown on or it may be applied to the paper as has been explained in connection with the wrapping paper. If the paper in between the design is not desired it can be removed easily and even burned out so that only the metal remains and the embossing of the design can take place right after if it is desired. This method is to be chosen when it deals of such decorations that must be nailed or tacked on or otherwise affixed to the objects that are to be ornated therewith. If it deals, however, with such decorations that cannot be nailed on and which must be painted on or at least applied through decalcomania whereby the bronze is already on the printed sheet, it is necessary to bronze first the so-applied design and to flux it whereupon the molten metal must be blown on. A device that serves in this respect is illustrated in Figure 6 and consists of the container 15 of the molten metal and the pipe through which acetylene or other burning hot gases are blown and which while rushing past the lowermost aperture of the container 15 entrain the molten metal and vaporize it and spray it against the object to be coated with the metal. The acetylene gas is chosen for its great heat that keeps the metal fluent while it is blown against the object that is to receive the coating. The paper may be made wet on its back so that it will not catch fire. The so-blown-on metal will stick only to those parts that are bronzed and consequently all the other parts can be cleaned easily from the sprayed-on metal. Objects that are made of materials that could burn must be held further away than those that will not catch fire.

Referring to the details of Figure 5, the paper roll as it comes from the paper mill is indicated by 12, the paper strip unrolled from that roll 12 is indicated by 10'. This paper 10' is moved along guides and over various cylinders. One of them, indicated by 16, is the cylinder that applies the lacquer or varnish to the underside of the paper 10' and the cylinder 17 contacts with the cylinder 16 and is partly immersed in liquid lacquer or varnish that is contained in the trough 18. The cylinder 19 serves for pressing the paper 10' on

the cylinder 16. The various cylinders revolve in the direction that is indicated by their arrows. The next cylinder 20 which is contacted by the paper 10' is the one that applies the bronze and it contacts with the powdered metal in the trough 21. The cylinder 22 may press the sheet 10' only slightly against the cylinder 20. There is also a duster 23 employed for removing the loosely hanging-on bronze. This duster consists of a cylindrical body that is covered with soft cloth 10 and it may revolve quicker than the other cylinders or in the direction that is inverse to that of the cylinder 20. There may be several dusting cylinders employed. The cylinder 24 applies the flux to the bronzed side of the paper 10' and is therefore immersed in liquid or semi-liquid flux in the trough 25. The cylinder 26 serves for pressing the paper 10' against the cylinder 24. Cylinders 27 and 28 serve for evening out the flux so that only very little is left on the bronzed paper 10'. The cylinder 29 that is partly immersed in the molten metal in the trough 30 applies that metal in form of a coating which will then be fused with the bronze on the paper 10'. This cylinder may be properly electrically heated 25 in order to keep the metal fluent that sticks to its cylindrical surface. As soon as the metal has cooled down somewhat and has therefore settled, the paper can be cut at 31 into large sheets 32 which are then ready for the printing press in 30 which the labels will be printed on the side that does not have any metal coating. It is obvious that the wrapping paper can be employed also in such way that the side with the metal coating will be the outer side of the wrapping while the 35 non-coated side of the paper may be the inside whereby the label may be embossed on the coated side, that is, on the metal. There may be as well both sides coated with the metal whereby one side may receive a different metal than the other. 40

In a somewhat similar manner could be coated those strips or sheets from which will be made the decorative parts that must be nailed or tacked or otherwise affixed to the objects that will be decorated therewith. In this instance, the various ornaments or figures, etc. must be printed on the paper 10' and in this case it could be the cylinder 16 whose cylindrical surface would have the drawing in elevated form as at 45 so that the varnish or lacquer would be applied only to the 50 elevated parts 45 on that cylindrical surface of the cylinder 16 and the impression upon the paper 10' would show the drawing that is shown in reverse by the elevated parts on the cylindrical surface of the cylinder 16. The impression on the sheet 10' or on already cut sheets could as well be performed on the regular printing press, either the lithographic or the type press. If the printing will be performed on the cylinder 16 there should be associated such parts 46 and screws 47 that permit the mounting of the aluminum plates or zinc plates 48 on the cylindrical surface of the cylinder 16 as is done also with the lithographic offset press. In addition there should also be employed the rollers for moistening the plate and 60 for the rolling on of the varnish. It will be, however, more simple to use the method as employed in the type presses where no moistening will be necessary. This is in so far important because there will no bronze stick to parts of the 70 sheet that are not printed on because there will not be any moisture thereon and since the operation is fast there is not enough time left for letting the sheet dry sufficiently before the bronze is applied to it. If the decorative parts have to 75

be embossed, which in most cases is necessary so that the design will be emphasized or that certain textures will be obtained as, for instance, on imitation shingles or bricks or on ledges, etc., there must be two more cylinders 33, 34 employed that must have the diameter of the cylinder 16 so that the embossed parts correspond exactly with the printed-on design. On the cylinder 33 will be mounted the steel sheets or forms that will be so cast or worked on (engraved, etc.) that the design will appear in embossed form on the sheet 10'. The cylinder 34 will exert the counter-pressure against the upper side of the paper 10' and the general design but not in a finished shape is also contained on a steel sheet that is laid on the cylindrical surface of the cylinder 34 whereby, however, the design is inverse to that of the steel sheet of the cylinder 33, that is to say, that the larger elevations on the steel sheet on cylinder 33 are made as depressions on the steel sheet of the cylinder 34 while larger depressions on the steel sheet of the cylinder 33 are formed as corresponding elevations on the steel sheet on the cylinder 34 so that the impressions simultaneously exerted by both steel sheets create the desired embossing as usually obtained in that art.

It is thus shown that with a machine which is shown in diagram in Figure 5, the finished product is delivered at the one end of that machine. Since the various plates and steel sheets can be replaced by others that have different designs, there may be different subjects printed and covered with metal and if desired also embossed. It is evident that this machine will serve also for making the wrapping paper as referred to before or the paper that serves for boxes, containers, etc. In this case only the plates around the cylinders need to be changed, that is, replaced as well as the steel sheets if no embossing is to be done.

The operation of the machine may in the simplest manner be accomplished through an endless chain 35 that is moved in the same ratio of speed as the paper 10'. Chain 35 is moved through the cog wheel 36 which is driven by a belt 37 that is driven by the motor 38 or by any conceivable suitable device that imparts motion. The chain 35 engages teeth that are circumferentially arranged on the one end of the cylinders 16, 20, 24, 29 and even on the cylinder 40 that serves for printing on labels or other descriptive or illustrative matter. The chain 35 is also laid around the cog wheel 41. There may be devices for lifting the paper 10' that is situated above the cylinder 29 in case in which the machine will be stopped and in order to prevent the burning of the paper 10'. Furthermore, there may be knives so arranged on the various cylinders that they will take off the excess amount of materials such as varnish, bronze, flux and molten metal and to thereby even out the amount of these materials so as to apply them evenly to the paper 10'. On decorative work where no paper is wanted at all the same can be burned away after the embossing is done.

It is clear that a number of details have been left away, especially those that belong to the mechanism for operating the machine, but having outlined the function the addition of the missing parts is only of secondary importance and they are left away in order that they do not obscure the diagram of the machine. Galvanization will not be employable to advantage and at 75 a lower cost with the materials aforesaid and

consequently it cannot substitute the process set forth above.

Having described my invention, what I claim is:

1. The method of coating dry materials with a layer of solid metal that sticks to them, comprising applying a sticky substance to said materials in any of the usual ways and with suitable implements, to the parts of said materials that are to be covered with said layer of solid metal, then bronzing these parts with powdered metal, 5 fluxing the bronzed parts and finally applying metal in molten condition to the bronzed parts by the use of suitable mechanical means, thus fusing said molten metal to the powdered metal in any desirable thickness and formation and 10 after having cooled off constituting said layer of solid metal.

2. The process of applying a layer of solid metal on a material that serves for enclosing goods that must be protected from the influence 20 of air and moisture; first, by rolling a sticky substance on said material thereby coating the latter with said substance, secondly, by covering said substance, while it is still sticky, with a layer of powdered metal so that the latter sticks to said 25 substance, third, by sparingly fluxing that layer of powdered metal and fourth by rolling a layer of said first named metal while in molten condition upon the layer of powdered metal, thus fusing said first named metal to said powdered 30 metal layer and leaving those parts on said material free that have not been covered with said sticky substance and the powdered metal.

3. The process of covering wrapping paper with a layer of solid tin, by printing a layer of 35 varnish to the paper, then powdering the so varnished side of the paper with powdered metal, then fluxing the powdered metal on the varnished side of the paper and finally rolling molten tin thereon, thus insuring the necessary evenness 40 and equal distribution of the solid tin over the whole paper besides the fast operation of these steps.

4. The process of creating layers of solid metal for decorative purposes whereby no liquids must 45 come in contact with the object to be so decorated, first, by making a layer of a sticky substance on that part of said object that is to be covered with said metal, then by bronzing that part with powdered metal, and by fluxing said bronzed 50 part and finally by laying molten metal thereto, thus fusing that metal to said powdered metal and after having cooled off constituting said layers of solid metal.

5. The process of decorating dry materials with 55 a layer of solid metal, by painting on said materials with an adhesive substance that is sticky when in wet condition and which is not soluble in water, then by powdering the so painted parts with powdered metal so as to cover the painted-on 60 substance and letting the powdered metal stick to it in form of a layer, then by fluxing said layer of powdered metal and finally by blowing molten metal upon said fluxed layer of powdered metal, thus fusing said molten metal with the powdered 65 metal and after having cooled down forming thereby said layer of solid metal.

6. The process of covering dry materials with a layer of solid metal, by applying bronzed parts to said dry materials through decalcomania where- 70 by the parts to be transferred are already bronzed, furthermore by fluxing the so transferred bronzed parts and then by applying molten metal to said bronzed parts either by blowing or by rolling it on the transferred bronzed parts if the shape of 75

- said dry materials permit the latter manipulation, thus fusing said molten metal to said bronzed parts and after having cooled off constituting said layer of solid metal.
5. 7. The process of printing a layer of solid metal on a suitable material such as paper, first, printing a substance thereon that is sticky when in wet condition and powdering that printed-on substance with powdered metal until it covers said substance entirely and thereby forms a layer of powdered metal that sticks to said substance then fluxing said powdered metal layer and printing a layer of molten metal upon the layer of powdered metal thus fusing the latter to said powdered metal layer and after having cooled off constituting said layer of solid metal.
8. The process of making decorations in form of solid metal, first by printing a sticky substance on a paper, whereby parts of said paper are left free from said substance, then by powdering the parts covered with said substance with powdered metal until a layer of powdered metal covers and sticks to said printed on substance, then by fluxing the layer of powdered metal and rolling a layer of molten metal on said powdered and fluxed metal thereby fusing it with said layer of powdered metal, and finally by removing the parts of the paper not covered with said layer of metal.
9. In a process for making solid metal parts for decoration and other purposes, first, of applying a sticky substance on a paper in form of a suitable decoration, lettering or any other design, then powdering said substance with powdered metal so that it sticks to said substance and thus forms a layer, then fluxing said layer of powdered metal and fusing molten metal to said layer of powdered metal and finally removing all the paper so as to leave only the foil or layer of the solid metal.
40. 10. A wrapping paper partly consisting of a paper that is unchanged in its appearance from the original finished state, an originally sticky substance evenly distributed on one side of that paper, a layer of powdered, fluxed and evenly distributed metal sticking to said substance and a layer of solid metal fused and sticking to said powdered metal layer.
11. A wrapping consisting of a paper that is unchanged in its evenness from its original finished state, having an evenly distributed originally adhesive substance sticking thereto on both sides, a layer of powdered and fluxed metal sticking to said substance on both sides of said paper and evenly distributed layers of solid metal fused and sticking to said layers of powdered metal.
12. A paper, even and unchanged from its original finished state, an evenly distributed originally adhesive substance sticking to said paper on both sides thereof, a layer of evenly distributed, powdered and fluxed metal sticking to said substance on both sides of said paper and another evenly distributed layer of solid metal, different in kind from the first named solid metal, fused to the powdered and fluxed metal on the other side of the paper.
13. The method of applying a layer of solid metal to smooth or rough surface metal, by making a layer of a sticky substance (paint etc.,) thereon, then by bronzing that sticky substance, then by fluxing the bronzed parts and finally by applying molten metal to the bronzed and fluxed parts.
14. The method of securing a layer of solid metal on a smooth surface of a dry material, by printing a sticky substance to said material, dusting (bronzing) that substance with powdered metal, fluxing the bronzed parts and applying molten metal to the bronzed and fluxed parts.
15. The method of securing a layer of solid metal on a material with a smooth surface like that of a mirror, glass, enamel, china and without the necessity of roughening or heating that surface, first by applying a sticky substance to said surface, then by powdering that substance with powdered metal, then by fluxing that powdered metal and finally by applying molten metal to the powdered metal, thus fusing the latter with said molten metal which constitutes the said layer of solid metal after it has cooled off.
16. Wrapping paper consisting partly of a sheet of paper that is still in its original finished state, said paper covered by a layer of solid metal of any suitable kind, the layer of solid metal fused to a base of fluxed powdered metal also of any suitable kind and that powdered metal sticking to an originally adhesive substance that is evenly distributed on said paper and that sticks thereto.
17. Wrapping paper consisting of a sheet of paper that is unchanged in its evenness from its original finished state and having a layer of solid metal of any suitable sanitary kind fused to a base of fluxed powdered metal of any suitable kind and that powdered metal sticking to varnish on said paper.
18. A waterproof material, such as, shingles, wall coverings for houses and other structures, having a core of fibrous material, such as, a sheet of paper or of cardboard, said fibrous material covered by a layer of solid metal of any suitable kind that is fused to a base of fluxed powdered metal of any suitable kind and that powdered metal sticking to an originally adhesive substance on that fibrous material and said substance sticking to said fibrous material.

HEINRICH KARL.